# EUROPEAN PATENT APPLICATION

(11) **EP 1 193 547 A1**
(43) Date of publication of application: **03.04.2002**
(21) Application number: 00925769.2
(22) Date of filing: 27.03.2000
(51) Int. Cl.: G03C 7/20, G03C 1/26

(54) **COLORED SPECTROZONAL SILVER-HALIDE PHOTOGRAPHIC MATERIAL**

(30) Priority: 01.02.2000 RU 2000102205
(71) Applicant: Zakrytoe Aktsionernoe Obschestvo Ordena Trudovogo Krasnogo Znameni Nauchno-Proizvodstvennoe Obiedinenie "Fomos" (ZAO NPO..., Moscow, 125167 (RU)
(72) Inventor: GRASHINA, Nataliya Alexandrovna, Moscow, 115516 (RU); GUSEVA, Ira Alexandrovna, Moscow, 117261 (RU); LIFSHITS, Eleonora Borisovna, Moscow, 125319 (RU); USHOMIRSKY, Mikhail Nikolaevich, Moscow, 111324 (RU); CHEKANOV, Valentin Vasilievich, Moscow, 105077 (RU)
(74) Representative: von Füner, Nicolai, Dr.
(86) International application number: RU0000103
(87) International publication number: WO0157593

(57) **Abstract**

The invention relates to area of colour photographic materials for registration of a colour image in visible and infra-red area.

The material comprises an antihalo backing layer on the one side of a polymer support and at least two light-sensitive layers prepared from silver halide emulsion, including colour forming couplers and sensitizing dyes, auxiliary and protective gelatin layers on the other side of the polymer support, said light-sensitive layers are prepared from silver bromide-iodide emulsion with octahedral or flattened microcrystals with an average size of the grain 0,5-1,5 µm or from their mixture and one light-sensitive layer contains as infra-red sensitizing dye one or more compounds of the formula where A = H, A¹ = OCH₂CH₂CH₂SO₃⁻, O - lower alkyl, A and A² together = CH₂C-(CH₃)₂CH₂ ⁻, A² = H, lower alkyl, B = H, 5,5 '-di-OCH₃, 6,6'-di-SCH₃, R = lower alkyl, (CH₂)₃SO₃⁻, n = 0,1; X = CH₃C₆H₄ SO₃⁻, J,-CH₃SO₃⁻, the alkaline metal or is absent; the second light-sensitive layer contains as orthochromatic sensitizing dye more than one compounds of the formula where Y = 0, N, A = lower alkyl or is absent, A¹ = H, lower alkyl, B = 5,5'-COOC₂H₅, 5,5'-C₆H₅, R, R' = lower alkyl, (CH₂)₃SO₃⁻, [K] ⁺ = NHC₅H₅ or is absent
and /or the third light-sensitive layer contains as panchromatic sensitizing of dye one or more compounds of the formula where A= lower alkyl, B = 4,5-benzo, 4,5-thieno, B¹ = 5-OCH₃, 5-C₆H₅, 4',5'-benzo, 5-Cl, 5-CH₃ ; R, R¹ = lower alkyl, (CH₂)₃SO₃⁻, [K]⁺ = HN (C₂H₅)₃, HN(C₄H₉)₃, C₅H₅-NH, the alkaline metal, 3,3'-diethylthiazolynecarbocyanine, or is absent, and between light-sensitive layers auxiliary gelatin layers including hardener are coated.

In addition the light-sensitive layers can contain activators of spectral sensitization.

The auxiliary gelatin layers can include derivatives of triazine-1,3,5 as a hardener.

It is desirable to add into light-sensitive layers a mixture of silver bromide-iodide photographic emulsions with octahedral microcrystals and with flattened microcrystals in the ratio 1:9-9:1.

The material according to the invention has a high resolving power (R = 110-160 mm⁻¹), i.e. in 1,6-2,3 times higher, than prototype, and more high light sensitivity.

## Description

This invention relates to a light-sensitive silver halide colour photographic materials for registration of objects in visible and infra-red area of a spectrum.

It is known the colour photographic material consisting from triacetate support coated thereon silver halide emulsion layers sensitive to various zones of a spectrum (TU 6-17-688-85 "Aerial photographic film, type SN-6M, NPO "Svema").

The indicated photographic material has a low resolving power R_{k=1,0} = 58 mm⁻¹.

It is known also a false colour silver halide photographic material consisting from a nitrate cellulose sublayered support having coated thereon on the one side a green anti-halo backing and on other side sequentially the first silver halide emulsion layer comprised silver bromide-iodide emulsion with the grain average size d=1,2µm and the contents of AgJ of 3 Mole %, containing 5-methyl-7-oxy-1,3,4-triazoindolizine (F-1) as a stabilizer, pyrocatechin, 3,3,9-triethyl-5,5'-diphenyloxacarbocyanine nitrate and 3,3'-diethyl-5-phenyl-5,6,9-trimethyloxathiacarbocyanine perchlorate as sensitizers, a yellow colour coupler (Zh-4) [4-stearoylaminobenzoyl acetic acid 2'-(3',5'-dicarboxyphenoxy)-5'-carboxyanylide, sodium salt of di-2-ethylhexyl ether of sulfosuccinic acid as a surfactant; the second silver halide layer prepared from same emulsion as the first layer and containing the same stabilizer F-1, pyrocatechin, sensitizer trietylamine salt of 3-ethyl-3'-γ-sulfopropyl-4-keto-4',5'-diphenyl-5-(3"-y-sulfopropyl-4",5"-diphenylthiazolidene-2"-ethylidene) thiazolinothiazolcyanine betaine and 3,3'1,9-triethyl-4,5,4',5'-dibenzothiacarbocyanine bromide as a sensitizer, as well as magenta colour coupler 1'-(4'-diphenoxy-3'-sulfophenyl)-3-heptadecylpyrazole-5-one, dipotassium salt of diether of a mixture of polyglycerides of alkenyl succinic acids as a surfactant; the third silver halide emulsion layer prepared from ammoniac silver bromide-iodide photographic emulsion with 3 Mole % of AgI and with the grain average size d = 1,0 µm containing stabilizer F-1, pyrocatechin, 3,3'-diethyl-10-methyl-5,5'-dimethoxy-6,6'-di-(methylmercapto) thiadicarbocyanine-n-tolusulfonate as a sensitizer, a cyan colour coupler 2'-methylotadecylamino-5'-sulfoanylide of 1-oxy-2-naphtoic acid (G-2), dipotassium salt of diether of mixture of polyglycerides of alkenyl succinic acids as a surfactant; protective layer containing gelatin, emulgate of 2,5-ditret-amylhydrochinone, phenol, surfactant (A. N. Iordanski "New false colour negative films", Journal of a Scientific and Applied Photography and Cinematography, volume 9, page 210-211, 1964). This material has a sensitivity S_{0,85} = 50 GOST, contrast coefficient 1.7-2.4, Dₘₐₓ > 2,5 for all layers, Dₒ = 0,11, resolving power R_{c=1,0} = 68 mm⁻¹ (GOST 9160-59).

It should be refer to defects of this material an insufficient level of a resolving power and photographic sensitivity not allowing to decode reliably small objects on photographies shot from large altitudes and from space, as well as a possibility of processing only at low temperatures.

An object of this invention is to provide an extension of a range of high sensitive false colour photographic materials with a sufficient level of a resolving power.

### Detailed description of the invention

The object of the present inventions accomplished with the false colour silver halide photographic material which comprises a polymeric support having coated thereon on the one side antihalo backing layer, on the other side at least two light-sensitive layers prepared from silver halide photographic emulsion, containing colour couplers and infrared, orthochromatic and/or panchromatic sensitizing dyes; auxiliary and protective gelatin layers; all sensitive layers are prepared from the silver bromide-iodide emulsion with octahedral or flattened microcrystals with a grain average size 0,5-1,5 microns, or from their mixture; one of the sensitive layers contains as infrachromatic sensitizing dye one or more one compounds represented by the general formula (I) wherein A represents H; A¹ represents OCH₂CH₂CH₂SO₃ ; O=lower alkyl; A and A¹ together represent CH₂C(CH₃)₂CH₂ ; A² represents H, lower alkyl; B represents H, 5,5'-di-OCH₃, 6,6'-di-SCH₃; R represents lower alkyl, (CH₂) ₃SO₃⁻ ; n = 0,1; X represents CH₃SO₃C₆H₄SO₃⁻, J, CH₃SO₃ -, the alkaline metal or is absent; other light-sensitive layer contains as an orthochromatic sensitizing dye more than one compounds of the formula (II) wherein Y represents 0, N; A represents lower alkyl or is absent; A¹ represents H, lower alkyl; B represents 5,5'-COOC₂H₅, 5,5 '-C₆H₅ ; R, R¹represent lower alkyl, (CH₂)₃SO₃⁻; [K]⁺ represents NHC₅H₅ or is absent, and/or the third light-sensitive layer contains as a panchromatic sensitizing dye one or more compounds of the formula (III) wherein A represents lower alkyl; B represents 4,5-benzo, 4,5-tieno; B¹ represents 5-OCH₃, 5-C₆H₅, 4,'5' -benzo, 5-CH₃, 5-Cl; R, R¹ represent lower alkyl, (CH₂) ₃ SO₃⁻ ; [K]⁺ represents HN(C₂H₅)₃, HN(C₄H₉)₃, C₅H₅-NH, the alkaline metal, 3,3'-diethylthiazolinocarbocyanine or is absent, and between light-sensitive layers auxiliary gelatin layers including hardener are coated.

In addition the light-sensitive layers can contain 3,3'-[1",2"bis(ethoxy)-ethyl]-bis-(1-ethylbenzimidazolium) diperchlorate, or disodium salt of 4,4'-bis(4",6-diphenoxy-1,3,5-triazynil-2-amino)stilbene-2,2'-disulfonic acid or monosodium salt of 2-mercaptobenzoxazole-5-sulfonic acid as an activator of the spectral sensitization.

As a hardener it is desirable to apply derivatives of triazine-1,3,5, namely: 1,3,5-triacryloylhexahydrotriazine or sodium salt of 2,4-dichloro-6-oxytriazine-1,3,5.

It is desirable to introduce in the light-sensitive layers mixtures of silver bromide-iodide emulsion with octahedral microcrystals and silver bromide-iodide emulsion with flattened microcrystals in the ratio 1:9-9:1.

As magenta colour couplers preferably derivatives of pyrazolone-5 and/or aminobenzenesulfamino-1,2-xylene are used: 1-(4-phenoxy-3-sulfophenyl)-3-stearoylamino-pyrazolone-5 (P-6), 3,5-di(2-methyl-5-octadecenyl-succinoylaminobenzenesulfamino)-1,2-xylene [P-8], 1-(2,4,6-trichlorophenyl)-3 [2,4-di-tret-amyl-phenoxy-acetylamido)-benzamido]-pyrazolone-5 (ZP-24), 1-(4'-phenoxy-3'-sulfophenyl) -3 -heptadecylpyrazolone-5 (P-1), 1-(2',4',6'-trichlorophenyl)-3[2"chloro-5"-octadecylsuccinoyliminophenyl]aminopyrazolone (N-651).

As cyan colour couplers preferably derivatives of 1-oxy-2-naphtoyl acid are used. Among such compounds are the following: 2-methyl-octadecylamino-5-sulfanilide of 1-oxy-2-naphtoyl acid (G-2), (2,4-di-tret-amylphenoxy)-bulylamide of 1-oxy-2-naphtoyl acid (ZG-97), octadecylamide of 1-oxy-4-sulfo-2-naphtoyl acid (G-3).

As yellow colour couplers preferably anylides of acylacetic, pivaylacetic or benzoic acids are used: 3,5-dicarboxyanylide of n-stearoylaminobenzoylacetic acid (Zh-2), 2-chloro-5 [γ-2,4-di-tret-anilid(phenoxy)-butyroylamino)-anilide]-α-n-carboxyphenyloxypivaylacetic acid (N-596), 2-chloro-5 [γ-2,4-di-tret-amyl(phenoxy)-butyroylamino)-anilide] of α-n-carbomethoxyphenoxypivaylacetic acid (N-574), 2'-methyloctadecylamino-5'-sulfanilide of benzoylacetic acid (Zh-8), 2'-chloro-5' (3", 5"-dicarboxyphenylsulfamydo)anilide of 2-octadecyloxybenzoylacetic acid (N-353), 2-chloro-5[(γ-2',4'-di-tret-amylphenoxy) (butyroylamino)anilide of α-benzylhydantoylpivaylacetic acid (Y-488), 2"-chloro-5" (3", 5"'-dicarbmethoxyphenylsulfamido)anilide of α-(3', 5'-dicarbmethoxyphenoxy)2-octadecyloxybenzoylacetic acid (N-609).

The false colour photographic material according to this invention expands essentially a range of high sensitive (S_{0,85} = GOST 200-700) materials with adequately high level of a resolving power (R = 100-145 mm⁻¹).

The following examples illustrate this invention, but do not limit it.

### Example 1 (the prototype).

False colour silver halide photographic material is prepared by coating on the undercoated nitrate cellulose base an emulsion and auxiliary layers of a following structure:
- Green antihalo sublayer from a mixture of isobutanol, propanol, novamal, BRO-721 dye and dimethylphtalate;
- Gelatin sublayer containing per 1 L of desalinated water 40 g of gelatin, 30 ml of the 4% solution of sodium salt of di-2-ethylhexyl ether of sulfosuccinic acid as a surfactant;
- The first silver halide emulsion layer containing silver bromide-iodide emulsion with an average grain size of 1,2 µm and AgJ content 3,08 %. The emulsion contains per 1 kg 40 ml of the 1% solution of F-1 5-methyl-7-oxy-1,3,4-triazoindolyzine as a stabilizer; 6 ml of the 1% solution of pyrocatechin, 40 ml of the 0,05% alcohol solution of 3,3', 9-triethyl-5,5'-diphenyloxacarbocyanine nitrate and 25 ml of the 0,05% alcohol solution of perchlorate 3,3'-diethyl-5-phenyl-5',6,9-trimethyloxathiacarbocyanine; 30 ml of the 5% solution of a yellow coupler (Zh-4) (2-(3,'5-dicarboxy-phenoxy-5'-carboxyanilide of 4-stearoylaminobenzoylacetic acid), 6 ml of the 4% solution of surfactant, dipotassium salt of diether of a mixture of polyglycerides of alcenylsuccinic acids;
- The second silver halide emulsion layer from the same emulsion as the first layer but containing per 1 kg of emulsion 40 ml of 0,05% alcohol solution triethylamine salt of 3-ethyl-3'-γ-sulfopropyl-4-keto-4',5'-diphenyl-5 (3"-γ-sulfopropyl-4",5"-diphenylthiazolynylydene-2"-ethylydene)thiazolinothiazolocyanine betaine and 30 ml of 0,1% alcohol solution of 3,3",9-triethyl-4,5,4",5'-dibenzothiacarbocyanine bromide as the spectral sensitizers and 200 ml of the 5% water solution of (P-1) 1-(4'-phenoxy-3"-sulfophenyl)-3-heptadezylpyrazolone-5 as a magenta coupler and 6 ml of the 4% solution dipotassium salt of a mixture of polyglycerides of alkenylsuccinic acids as surfactant;
- The third silver halide emulsion layer from silver bromide-iodide emulsion with an average grain size d=1,0 µm and contents of AgJ of 3 Mol. %, containing 40 ml of the 1% solution of a stabilizer F-1, 6 ml of the 1% solution of pyrocatechin, but including per 1 kg of emulsion 30 ml of 0,01% alcohol solution of 3,3'-diethyl-10-methyl-5,5'-dimethoxy-6,6-di-(methylmercapto- thiadicarbocyanine-*para*-tolusulfonate as a spectral sensitizer, 500 ml of the 3% solution of 2'-methyl-octadecylamino-5'-sulfoanilide of 1-oxy-2-naphthoic acid (G-2) as a a cyan coupler, 6 ml of the 4% solution of dipotassium salt of diether of a mixture of polyglycerides of alkenylsuccinic acids as a surfactant;
- a protective layer from the following composition: per 1 L of desalinated water 20 g of a gelatin, 20 g of 2,5-di-tret-amylhydrochinone, 8 ml of 4% solution of sodium salt of di-2-ethylhexyl ether of sulfosuccinic acid as a surfactant.

A film is exposed according to GOST 9160-91 at colour temperatures 3200 K and 5500K behind the filter ZhS-18, and processed according to TU 6-17-1372-89.

| **Mode of processing** | | | |
|---|---|---|---|
| No. | Processing stage | Duration time, min | Solution temperature, °C |
| 1 | Colour development | 5-10 | 25±3 |
| 2 | Bleaching-fixing | 10 | 23±1.0 |
| 3 | Washing | 5 | 25±1.0 |
| 4 | Drying | - | no less than 60 at the speed 100 m/h |

| Colour developer, g/L: | |
|---|---|
| Trilon B | 2,0 |
| Hydroxylamine hydrochloride (sulfate) | 2,0 |
| Ethyloxyethyl-paraphenylene diamine | 4,5 |
| K₂CO₃ | 75 |
| Na₂SO₃ anhydrous | 2,0 |
| KBr | 2,0 |
| Benzotriazole | 0,02 |
| Water | up to 1 L. |
| pH | 10,7±0,1 |

| Bleaching-fixing solution | |
|---|---|
| Trilon B | 10,0 |
| Na₂SO₃ anhydrous | 30,0 |
| KH₂PO₄ | 5,8 |
| NaHPO₄ | 4,3 |
| Na₂CO₃ anhydrous | 6,0 |
| Trilon B, iron salt | 60,0 |
| Thiosemicarbazide sulfate | 10,0 |
| Water | - up to 1 L. |

Photographic sensitivity is determined on a criterion S_{0,85} over a fog density on the formula S = K/H with a factor K = 20; a resolving power is determined according to GOST 2819-84.

The results of tests of this and all following examples are indicated in the table.

### Example 2 (comparative)

False colour photographic material is prepared by coating on two-side subcoated polyethylene terephtalate support of emulsion and auxiliary layers of the following structure:
- blue antihalo sublayer consisting from suspension of colloid silver, containing per kg 13.5 g of metal silver; 133 g of gelatin; 140 g of 2,5-ditret-octylhydrochinone; 150 ml of 4% solution of a mixture of sodium salt of diisobutylnaphtaline sulfonic acid and 30 ml of 4% water solution of disodium salt of diethyl ether of N-γ-dodecyloxypropyl(sulfosuccinoyl)aspartic acid as surfactants; 60 ml of the 3% solution of sodium salt of 2,4-dichloro-6-oxytriazine-1,3,5 as a hardener;
- gelatin sublayer containing per 1 L of desalinated water 40 g of and 30 ml of the 4% solution of sodium salt of di-2-ethylhaxyl ether of sulfosuccinic acid as a surfactant;
- the first silver halide emulsion layer prepared from polydispersional silver bromide-iodide emulsion (average grain size 0,5 µm, variation factor, Cγ = 35 %, metal silver 54 g/kg, AgJ 3 mole %, gelatin 7 %). It is added per 1 kg of emulsion: 40 ml of the 1% solution of F-1 5-methyl-7-oxy-1,3,4-triazoindolyzine as a stabilizer, 6 ml of the 1% solution of pyrocatechin, 60 ml of 0,1% alcohol solution of a spectral sensitizer of the formula (II) (Y = N, A = C₂H₅, A¹ = H, B = 5,5 '-COOC₂ H₅, R-= (CH)²SO₃, R¹ = C₂H₅, [K]⁺ - is absent); spectral sensitizer of the formula (II) (Y = O, A¹ = C₂H₅, B = 5,5'-C₆H₅, R, R¹ = (CH₂)₃SO₃, [K]⁺ = NHC₅H₅) in an amount of 30 ml of 0,1% alcohol solution; then it is added 160 ml of the 5% solution of 2'-methyloctadecylamino-5'-sulfoanilide of benzoylacetic acid (Zh-8) and 250 ml of 3% solution of 2'-chloro-5'-(3",5"-dicarboxyphenylsulfamido)anilide of 2-octadecyl-oxybenzoylacetic acid (N-353) as yellow couplers (ratio Zh8:N-353 = 1:1) and 10 ml of diluted nitric acid (1:30). Then it is added 40 ml of the 4% solution of sodium salt of di-2-ethylhexyl ether of sulfosuccinic acid and 10 ml of 0,1% solution of dipotassium salt of diether of a mixture of polyglycerides of alkenylsuccinic acids as surfactants and 20 ml of 3% solution of sodium salt of 2,4-dichloro-6-oxy-triazine-1,3,5 a hardener.

Gelatin sublayer has a following composition: per 1 L of desalinated water 40 g of gelatin, 120 ml of the 3% solution of a yellow coupler N-353, 20 ml of the 4% solution of sodium salt of di-2-ethylhexyl ether of sulfosuccinic acid and 10 ml of 0,1 M solution of dipotassium salt of diether of a mixture of polyglycerides of alkenylsuccinic acids as surfactants and 10 ml of the 3% solution of sodium salt of 2,4-dichloro-6-oxy-triazine-1,3,5 (DU-679) as a hardener.

The second silver halide emulsion layer is prepared from same emulsion, as a first layer. It is added peri kg of emulsion 40 ml of the 1% solution of a stabilizer F-1, 6 ml of 1% pyrocatechin, 30 ml of the 0,2% solution of diperchorate 3,3-[1",2"-bis(ethoxy)-ethyl]-bis-(1-ethylbenzimidazolium) as an activator of spectral sensitization, 80ml of 0,05% alcohol solution of spectral sensitizer of the formula III (A = C₂H₅, B = 4,5-benzo, B¹ = 5-OCH₃, R = (CH₂)₃SO₃⁻, R¹ =C₂H₅, [K ⁺] is absent), 600 ml of the 3% solution of 2-methyloctadecylamino-5-sulfoanilide-1-oxy-2-naphtoic acid (G-2) as a cyan coupler, 40 ml of the 4% solution of a sodium salt of di-2-ethyloxyl ether of a mixture of polyglycerides of alkenylsuccinic acids as a surfactant, 18 ml of the 3% solution of sodium salt of 2,4-dichloro-6-oxy-triazine-1,3,5 as a hardener. Gelatin interlayer is coated containing per 1 L of desalinated water 40 g of the 2% gelatin solution, 50 ml of the 4% solution of sodium salt of di-2-ethylhexyl ether of sulfosuccinic acid and 15 ml of 0,1 Mole solution of dipotassium salt of diether of a mixture of polyglycerides of alkenylsuccinic acids as surfactants and 10 ml of the 3% solution of sodium salt of 2,4 dichloro-6-oxytriazine-1,3,5 as a hardener.

The third silver halide emulsion layer is prepared from the same emulsion, as the other layers, but it is added per 1 kg of emulsion 40 ml of the 1% stabilizer F-1, 6 ml of 1% pyrocatechin, 75% of 1% alcohol solution of disodium salt of 4,4'-bis(5,6-diphenoxy-1,3,5-triazinile-2-aminostilbene-2,2'-disulfonic acid as an activator of sensitization; 45 ml of 0,02% alcohol solution of sensitizing dye of the formula I (A, A¹ together -CH₂C(CH₃)₂CH₂, A² = CH₃, B = 5,5'-di-OCH₃, 6,6'-di-SCH₃, R = C₂H₅, X = CH₃C₆H₄SO₃⁻, n = 0); 15 ml of 0,03% alcohol solution of sensitizing dye of the formula I (A, A² = H, A¹ = OCH₂CH₂CH₂CH₂SO₃⁻, B = H, R = C₂H₅, n = 1, X - is absent), 5 ml 0,5% solution of 2-heptyl-5-methyl-7-oxy-1,3,4-triazine indazine, mixture of [1-(4-phenoxy-3-sulfophenyl)-3-stearoylaminopyrazolone-5] (P-6) and 3,5-di-(2-methyl)-5-octadecenylsuczinoylaminobenzenesulfamino)-1,2-xylene (P-8) as magenta couplers in the ratio of P-6:P-8 = 4:1, in amount of 350 ml of the 5% solution, 40 ml of 4% solution of sodium salt of di-2-ethylhexyl ether of sulfosuccinic acid and 10 ml of 0,1 Mole solution of dipotassium salt of diether of a mixture of monoglycerides of alkenylsuccinic acids as surfactants, 20 ml of the 3% solution of sodium salt of 2,4-dichloro-6-oxytriazine-1,3,5 as a hardener.

A protective layer is coated with the following composition: per 1 L of desalinated water it is added 40 g of gelatin, 20 ml of the 4% solution of sodium salt of di-2-ethylhexyl ether of sulfosuccinic acid and 10 ml of 0,1 Mole solution of dipotassium salt of diether of a mixture of polyglycerides of alkenylsuccinic acids as surfactants, 50 ml of 5 % solution of a mixture of magenta couplers P-6 and P-8 in the ratio P-6:P-8 = 4:1, 20 ml of the 3% solution of sodium salt of 2,4-dichloro-6-oxytriazine-1,3,5 as a hardener.

A film is exposed and processed as in an example 1. The properties are represented in the table.

### Example 3.

False colour photographic material is prepared and processed similarly to the example 2, but all light-sensitive silver halide emulsions contain a mixture of two emulsions: silver bromide-iodide emulsion with octahedral microcrystals with average grain size 0,7 µm and silver bromide-iodide emulsion with flattened microcrystals (aspect ratio 1:5) with average grain size 1,2 µm; in protective and auxiliary gelatin layers the colour couplers are not added.

### Example 4.

False colour photographic material is prepared and processed similarly to the example 2, but an interlayer is coated only on the first light sensitive silver halide emulsion layer; into the second layer 700 ml of the 3% solution of a cyan coupler G-2 and 25 ml of the 3 solution of sodium salt of 2,4-dichloro-6-oxytriazine-1,3,5 as the hardener are added; in the third light-sensitive layer 80 ml of 0,02% alcohol solution of a sensitizing dye of the formula I (A, A¹ together - CH₂C (CH₃)₂CH₂, A² = CH₃, B = 5,5'-di-OCH₃, 6,6'-di-SCH₃, R = C₂H₅, X⁻ = CH₃C₆H₄SO₃⁻, n = 0), is added.

### Example 5 (comparative)

False colour silver halide photographic material is prepared by coating on two-side sublayered polyethylene terephtalate support of the emulsion and auxiliary layers of the following structure:
- blue antihalo backing layer from a colloid silver suspension containing per kG of emulsion 13,5 g of metal silver, 133 g of gelatin, 140 g of 2,5-di-tret-octylhydrochinone, 150 ml of the 4% solution mixture of sodium salts of diisobutylnaphtalene sulfonic acid and 30 ml of the 4% solution of disodium salt of diethyl ether of N-γ-dodecyloxypropyl-(sulfosuccinoyl)-asparagine acid as surfactants, 45 ml of the 3% solution of 1,3,5-triacryloylhexahydrotriazine as a hardener, desalinated water up to 1 L;
- gelatin sublayer containing per 1 L of desalinated water 40 g of gelatin, 30 ml of 4% solution of sodium salt of di-2-ethylhexyl ether of sulfosuccinic acid as a surfactant;
- the first light-sensitive silver halide emulsion layer is prepared from polydispersional silver bromide-iodide emulsion (average size of microcrystals d = 0,7 µm, Cᵥ = 30 %, contents of AgJ 3 Mole %) containing per 1 kg emulsion 40 ml of the 1% solution of 5-methyl-7-οκc -1,3,4-triazoindolizine, 6 ml of the 1% solution of pyrocatechin, 100 ml of 0,05% alcohol solution of 3,9-diethyl-3-γ-sulfopropyl-5-methoxy-4,5-benzothiacarbocyaninebetaine as a spectral sensitizing dye, 600 ml of the 3% solution of 2-methyloctadecylamino-5-sulfoanilide-1-oxy-2-naphtoic acid (G-2) as a cyan coupler, 150 ml of the 3% solution of 3,5-dicarboxyanilide-n-stearoylaminjbenzoylacetic acid(Zh-2) as a yellow coupler (G-2:Zh-2 ratio = 4:1); 10 ml of 5% solution of cyan dye - product of oxidation of 1,2-naphtyldiamine-5,7-disulfonic acid with a chloric iron; 10 ml of the diluted nitric acid (1:30); 40 ml of 4% solution of the sodium salt of di-2-ethylhexyl ether of sulfosuccinic acid and 10 ml of 0,1 M solution of the dipotassium salt of diether of a mixture of polyglycerides of alkenylsuccinic acids as surfactants;
- gelatin interlayer containing per 1 L of desalinated of water 40 g of gelatin, 120 ml of the 5% solution of octadecylamide of 1-oxy-4-sulfo-2-naphtoic acid(G-3) as a cyan coupler, 30 ml of the 4% solution of the sodium salt of di-2-ethylhexyl ether of sulfosuccinic acid and 10 ml of 0,1 Mole solution of the sodium salt of di-2-ethylhexyltetraethylenglycol ether of sulfosuccinic acid as surfactants; and 15 ml of the 3% solution of 1,3,5-triacryloulhexahydrotriazine as the hardener.

The second light-sensitive silver halide emulsion layer is prepared from the same emulsion as the first layer, but it is added per 1 kg emulsion 110 ml of the 1% solution of disodium salt of 4,4'-bis-(4,6-diphenoxy-1,3,5-triazynil-2-amino)stilbene-2,2'-disulfonic acid as supersensitizer; 60 ml of 3,3'-diethyl-10-methyl-5,5'-dimethoxy-6,6'-di(methylmercapto)thiadicarbocyanine-n-tolusulfonate as a spectral sensitizer; mixture of magenta couplers P-6 and P-8 in a mass ratio 2:1 in an amount of 375 ml of the 5% solution; 20 ml of 4% solution of sodium salt of di-2-ethylhexyl ether of sulfosuccinic acid and 10 ml of 0,1 M solution of dipotassium salt of diether of a mixture of polyglycerides of alkenylsuccinic acids as surfactants.

The protective layer is coated from the next composition: per1 l of desalinated water 40 g of gelatin; 15ml of 4% solution of sodium salt of di-2-ethylhexyl ether of sulfosuccinic acid as the surfactant and 20 ml of the 3% solution of 1,3,5-triacroylhexahydrotriazine as the hardener.

The material is exposed and processed as in an example 1. The properties are indicated in the table.

### Example 6.

False colour photographic material is prepared similarly to the example 5, but in one of the light-sensitive emulsion layers it is added 20 ml of the 0,2% solution of diperchlorate of 3,3'-[1",2"-bis(ethoxy)-ethyl]-bis-(1-ethylbenzimidazolium) as the activator of the spectral sensitization and 8 ml of the 0,05% solution of sensitizing dye of the formula III (A = C₂H₅, B = 4,5-benzo, B¹ = 5-OCH₃, R = (CH₂)₃SO₃⁻, R¹ = (CH₂H₅, [K] ⁺ is absent), and 30 ml of the 3% solution of sodium salt of 2,4-dichloro-6-oxytriazine-1,3,5 as the hardener; in the gelatin interlayer a cyan coupler is not added.

In the other light-sensitive silver halide emulsion a layer it is added as a sensitizing dye a compound of the formula I (A, A¹ together = CH₂C(CH₃)₂CH₂, A² = CH₃, B = 5;5'-di-OCH₃, 6,6'-di-SCH₃, R = C₂H₅, X⁻ = CH₃C₆H₄SO₃⁻, n = 0) in an amount of 80 ml of 0,02% alcohol solution, 75 ml of the 1% solution of disodium salt of 4,4'-bis-(4,6-diphenoxy-1,3,5-triazinile-2-amino)stilbene2,2'-disulfonic acid as the supersensitizer and 6 ml of the 0,5% solution of 2-heptyl-5-methyl-7-oxy-1,3,5-triazaindolizine; then 350 ml of the 5% solution of a mixture of magenta couplers P-6 and P-8 in a mass ratio 4:1; 40 ml of the 4 % solution of the sodium salt of di-2-ethylhexyl ether of sulfosuccinic acid and 10 ml of 0,1 M of a solution of dipotassium salt of diether of a mixture of polyglycerides of alkenylsuccinic acids as surfactants and 15 ml of the 3% solution of sodium salt of 2,4-dichloro-6-oxytriazine-1,3,5 as the hardener. In the protective layer magenta couplers are not added.

A material is exposed and processed as in an example 1. The properties are represented in the table.

### Example 7.

False colour photographic material is prepared similarly to example 6, but all light-sensitive silver halide layers is prepared from a mixture of silver bromide-iodide emulsion with octahedral microcrystals with an average grain size 0,7 µm and silver bromide-iodide emulsion with flattened microcrystals with an average grain size 0,15 µm and aspect ratio 1:5 at emulsions ratio 9:1.

### Example 8.

False colour photographic material is prepared similarly to example 6, but in one light-sensitive layer it is added sensitizing dye of the formula II (A - C₂H₅, B - 4,5-benzo, B¹ = 5-OCH₃, R = (CH₂)₃SO₃⁻, R¹= C₂H₅, [K]⁺ - is absent) in an amount of 120 ml of the 0,05% solution, then 800 ml of the 3% solution of G-2 cyan coupler, 200 ml of the 3% solution of Zh-2yellow coupler; 60 ml of the 4% solution of sodium salt of di-2-ethylhexyl ether of sulfosuccinic acid and 20 ml of 0,1 M of a solution of dipotassium salt of diether of a mixture of polyglycerides of alkenylsuccinic acids as surfactants.

In the other light-sensitive layers it is added as sensitizing dye a compound of the formula (I) (A, A¹ together = CH₂C(CH₃)₂CH₂, A² = CH₃, B = 5,5'-di-OCH₃, 6,6'-di-SCH₃, R = C₂H₅, X⁻ = CH₃C₆H₄SO₃⁻, n = 0) in an amount of 100 ml 0,02% of alcohol solution and 8 ml of the 0,5% solution of 2-heptyl-5-methyl-7-oxy-1,3,4-triazaindolizine. A mixture of P-6 and P-8 magenta couplers (in a mass ratio 4:1) is added in an amount of 400 ml of the 5% solution.

### Example 9.

False colour photographic material is prepared similarly to example 5, but in one light-sensitive silver halide emulsion layer a sensitizing dye of the formula III (A = C₂H₅, B = 4,5-benzo, B¹ = 4',5'-benzo, R = R¹-(CH₂)₃SO₃⁻, [K]⁺ = C₅H₅N⁺H), in an amount 100 ml of 0,05% alcohol solution are introduced.

In the other light-sensitive silver halide layer as a sensitizing dye a compound of the formula I (A, A² = H, A¹ = OCH₂CH₂CH₂SO₃⁻, B = H, R = C₂H₅, n = 1, X is absent), in an amount of 30 ml of 0,03% alcohol solution and a compound of the formula I (A, A² together = CH₂C(CH3)₂CH₂, A² = CH₃, B = 5,5'-di-OCH₃, 6,6'-di-SCH₃, R = C₂H₅, X⁻ = CH₃C₆H₄SO₃⁻, n = 0) in an amount of 20 ml of 0,02% alcohol solution are introduced.

### Example 10.

False colour silver halide photographic material is prepared similarly to example 9, but all light-sensitive emulsion layers is prepared from silver bromide-iodide emulsion with flattened microcrystals with an average grain size 0,9 µm at the aspect ratio 1:5.

### Example 11.

False colour silver halide photographic material is prepared similarly to example 6, but as colour couplers a dispersion of cyan hydrophobic coupler (ZG-97) 2,4-(di-tret-amylphenoxy)-butylamide-1-oxy-2-naphtoic acid is introduced. A dispersion of a ZG-97 coupler is prepared in high pressure homogenizer according to the following prescription: ZG-97- 10 parts by weight, dibutylphtalate - 8 parts by weight, ethylacetate - 16 parts by weight, water solution of gelatin with a mass concentration 100 g/L - 65 parts by weight. An emulgator is used a water solution of sodium salt of dodecylbenzenesulfonic acid, 12 parts by weight and 0,3 parts by weight of oil-soluble surfactant;
a dispersion of a magenta coupler (ZP-24) 1-(2',4',6'-trichlorophenyl)-3-[(2",4"-di-tret-amylphenoxyacetamydo)-benzamido]-pyrazolone-5 is prepared on the next prescription: ZP-24 - 6 parts by weight, dibutylphtalate - 8 parts by weight, ethylacetate - 24 parts by weight, water solution of gelatin with mass concentration 60 g/L - 50 parts by weight, emulgator - 28 parts by weight;
yellow couplers N-596 (2-chloro-5-[(γ-2,4-di-tret-amylphenoxy)-butyroylamino)-anilide] of α-n-carboxyphenoxypyvaloylacetic acid) and N-574 (2-chloro-5 [(γ-2,4-di-tret-amylphenoxy)-butiroylamino)-anilide] of α-n-carbmethoxyphenoxypyvaloylacetic acid) is used as a joint dispersion, prepared in high pressure homogenizer on the following prescription: N-596 - 4 parts by weight, N-574 - 2 parts by weight, dibutylphtalate - 8 parts by weight, ethylacetate - 23 parts by weight, water solution of gelatin with mass concentration 80 g/L - 80 parts by weight, emulgator - 200 parts by weight;

In emulsion of one layer (per 1 kg of emulsion) is introduced 600 g of a dispersion of a coupler ZG-97 and 160 g of a joint dispersion of couplers N-596 and N-574(2:1).

In gelatin interlayer and protective layer a dispersion of a colour couplers is not added.

A material is exposed as in an example 1, but processed on the process of C-41 type, namely:

| **Mode of processing** | | |
|---|---|---|
| Processing stage | Processing stage duration, min | Temperature of solutions and washing water, °C |
| Development | 5-7 | 30.0±0.03 |
| Bleaching-fixing | 6-7 | 30±1 |
| Washing | 3 | 30±2 |
| Drying | | 40-60 |

### Example 12.

False colour silver is prepared from a mixture in the ratio 7:3of silver bromide-iodide emulsion with octahedral microcrystals, d = 0,7, and silver bromide-iodide emulsion with flattened microcrystals with aspect ratio 1:5.

### Example 13.

False colour silver halide photographic is prepared similarly to example 12, but in one emulsion layer it is added sensitizing dye of the formula (III) (A = C₂H₅, B = 4,5-thieno, B¹ = 6-OCH₃, 5-C₆H₅, R = R¹- (CH₂)SO₃⁻ [K] ⁺ = HN⁺(C₂H₅)₃) in an amount of 75,0 ml of 0,10% alcohol solution and monosodium salt of 2-mercapto-benzoxazole-5-sulfonic acid in an amount of 20 ml of the 0,05% solution as an activator of spectral sensitization.

In other emulsion layer as a sensitizing dye it is added compound of the formula I (A² -CH₃, A, A¹ together - CH₂C(CH₃)₂CH₂, B - 5,5'-di-OCH₃, 6,6 '-di-SCH₃, R - C₂H₅, X = CH₃C₆H₄SO₃ ⁻, n = 0) in an amount of 60 ml of 0,02% alcohol solution and the compound of the formula I (A,A² = H, A¹ = OCH₂CH₂CH₂SO₃⁻, B = H, R = C₂H₅, n = 1, X is absent)..

### Example 14.

False colour silver halide photographic material is prepared similarly to example 13, but all light-sensitive layers are prepared from silver bromide-iodide photographic emulsion with an average size of flattened crystals 1,5 µm at aspect ratio 1:5.

### Example 15.

False colour a photographic material is prepared similarly to example 13, but all light-sensitive silver halide emulsion layers are prepared from a mixture of silver bromide-iodide photographic emulsion with octahedral microcrystals with an average grain size d = 0,7 µm and silver bromide-iodide photographic emulsion with flattened microcrystals with d = 1.2 µm in the ratio 1:1.

### Example 16.

False colour silver halide photographic material is prepared similarly to example 15, but in one light-sensitive layer it is added as a sensitizing dye a compound III (A = C₂H₅, B = 4,5-benzo, B¹ = 5'-OCH₃, R = R¹-(CH₂)₃SO₃, [K⁺] = HN⁺ (C₄H₉)₃), in an amount of 120 ml of 0,1% alcohol solution and as an activator of spectral sensitization diperchlorate of 3,3'-[1",2"-bis(ethoxy)-ethyl]-bis-(1-ethylbenzoimidazolium) in an amount 45 ml of the 0,2% solution. Then 375 g of (5,7%) dispersion of a cyan coupler ZG-97 ((2,4-di-tret-amylphenoxy)-butylamide of 1-oxy-2-naphtoic acid) obtained on high pressure homogenizer on the following prescription: ZG-97 - 57,2 g, dibutylphtalate - 55 g, ethylacetate - 260 g, gelatin solution with mass concentration 60 g/L - 790 g, solution of emulgator with mass concentration 40 g/l - 98 g.

Also it is added 75 g of 6.2% dispersion of a yellow coupler N-596 ([2-chloro-5-[γ-2,4-di-tret-amyl(phenoxy)-butiroylamino)anilide of α-n-carboxyphenoxypyvaloylacetic acid), prepared on high pressure homogenizer according to the prescription: N-596 - 62,3g, tricresylphosphate - 31,2 g, N-azoamylphtalimide - 31,1 g, ethylacetate - 250 g, gelatin solution with mass concentration - 80 g/L - 779 g, solution of emulgator with mass concentration 40 g/L - 96,4 g.. As a hardener 20 ml of the 3% solution of sodium salt of 2,4-dichloro-6-oxy-triazine-1,3,5 is added.

Gelatin interlayer is prepared from a following composition: per 1 L of desalinated water 50 g of gelatin, 30 ml of 4% sodium salt of di-2-ethylhexyl ether of sulfosuccinic acid and 10 ml of 0,1 M solution of dipotassium salt of diether of a mixture of polyglycerides of alkenylsuccinic acids as the surfactants and 35 ml of the 3% solution of a hardener 1,3,5-triacryloylhexahydrotriazine are added.

In the other light-sensitive silver halide layer per 1 kg of emulsion it is added as a sensitizing dye 33 ml of 0,02% alcohol solution of compound of the formula I (A,A¹ together = CH₂C(CH₃)₂CH₂, A² = CH₃, B = 5,5'-di-OCH₃, 6,6'-di-SCH₃, R = C₂H₅, X = CH₃C₆H₄SO₃⁻ , n = 0) and before than sensitizing dye it is added 75 ml of the 1% solution of disodium salt of 4,4'-bis(4,6-dihenoxy-1-3-5-triazinyl-2-amino)stilbene of 2,2-disulfonic acid as a supersensitizer and 5 ml of the 0,5% solution of 2-heptyl-5-methyl-7-oxytriazaindolycine. Then 500 g of a dispersion of a magenta coupler (ZP-24) (1-(2,4,6-trichlorophenyl)-3[2,4-ditret-amyl-phenoxyacetylamido)-benzoamido]-pyrazolone-5) is added obtained on high pressure homogenizer according to the prescription: ZP-24 - 56 g, tricresylphosphate - 28g, N-isoamylphtalimide - 28 g, gelatin solution with mass concentration 60 g/L - 773 g, solution of emulgator sodium salt of dodecylbenzensulfonic acid with mass concentration 40 g/L - 115 g.

A protective layer is prepared from the composition: per 1 L of desalinated water 50 g of gelatin and 30 ml of 4% solution of sodium salt of di-2-ethylhexyl ether of sulfosuccinic acid and 10 ml of 0,1 M solution of dipotassium salt of diether of a mixture of polyglycerides of alkenylsuccinic acids as the surfactants and 30 ml of the 3% solution of sodium salt of 2,4-dichloro-6-oxytriazine-1,3,5 as a hardener.

### Example 17.

False colour silver halide photographic material is prepared similarly to example 16, but gelatin interlayer between light-sensitive layers is not introduced; in one light-sensitive layer it is added 490 g of a dispersion of cyan coupler ZG-97 and 145 g of a dispersion of a yellow coupler Y-488 (2-chloro-5-[(γ-2',4'-di-tret-amylphenoxy) butiroylamino)-anilide of α-benzylhydantoylpyvaloylacetic acid), obtained on high pressure homonizer according to the prescription: 69,7 g of a yellow coupler, 32 g of dibutylphtalate, 99 g of ethylacetate, 780 g of a gelatin solution with mass concentration 60 g/l, 119 ml of the 4% solution of sodium salt of dodecylbenzenesulfonic acid as an emulgator.

### Example 18.

False colour silver halide material is prepared similarly to example 16, but between light-sensitive layers a gelatin interlayer without colour couplers is coated. In other layer instead of a dispersion of a magenta coupler ZP-24 500 g a dispersion of a magenta couplers ZP-24 and N-651 is added, obtained as a joint dispersion prepared on high pressure homogenizer according to the prescription: 120 g of tricresylphosphate, 360 ml of ethylacetate, 2400 ml of a gelatin solution with mass concentration 60 g/L, 530 ml of an solution of a sodium salt of dodecylbenzensulfonic acid with mass concentration 40 g/L as an emulgator.

A protective layer contains per 1 L of desalinated water 55 g of gelatin, 30 ml of the 4% solution of sodium salt di-2-ethylhexyl ether of sulfosuccinic acid and 10 ml 0,1 M solution of dipotassium salt of diether of a mixture of polyglycerides of alkenylsuccinic acids as the surfactants and 34 ml of the 3% solution of the sodium salt of 2,4-dichloro-6-oxy-triazine-1,3,5 as a hardener.

### Example 19.

False colour silver halide photographic material is prepared similarly to example 2, but after spectral sensitizers in one layer it is added 570 g of a dispersion of a yellow coupler N-609 (2"-chloro-5"(3",5"-dicarbomethoxyphenylsulfamido)anilide of α-(3',5'-dicarbomethoxyphenoxy-2-octadecyloxybenzoylacetic acid) obtained on high pressure homogenizer according to the prescription: 207,5 g of N-609, 45 g of 2,5-di-tret-octylhydrochinone, 45 ml of tricresylphosphate, 1650 ml of gelatin solution with mass concentration 60 g/L, 260 ml of the 4% solution of sodium salt of dodecylbenzenesulfonic acid as an emulgator and 370 ml of ethylacetate.

In the other layer after spectral sensitizers it is added 490 g of a dispersion of a cyan coupler ZG-97 ((2,4-di-tret-amylphenoxy)butylamide-1-oxy-2-naphtoic acid) obtained on high pressure homogenizer according to the prescription: ZG-97 - 10 parts by weight, dibutylphtalate - 8 parts by weight, ethylacetate - 16 parts by weight, gelatin water solution with mass concentration 100 g/L - 65 parts by weight, water solution of sodium salt of dodecylbenzensulfonic acid -12 parts by weight, oil-soluble surfactant - 0,3 parts by weight.

In the third light-sensitive layer it is added after spectral sensitizers 540g of a joint dispersion of magenta couplers ZP-24 and N-651 prepared in high pressure homogenizer according to the prescription: 120 g of ZP-24, 60 g of N-651, 180 ml of tricresylphosphate, 360 ml of ethylacetate, 2400 ml of a gelatin solution with the mass concentration 60 g/L and 530 ml of sodium salt of dodecylbenzensulfonic acid as an emulgator.

In gelatin interlayers and protective layer the colour couplers are not added. A material is exposed and processed on process C-41, as in an example 11. The properties are represented in the table.

### Example 20.

False colour silver halide photographic material is prepared similarly to example 19, but all light-sensitive layers are prepared from a mixture of two emulsions: silver bromide-iodide emulsion with octahedral microcrystals with an average grain size d = 0,7 µm and silver bromide-iodide emulsion with flattened microcrystals (aspect ratio 1:5) with an average grain size 1,2 µm.

In the one light-sensitive layer it is added 660 g of a dispersion of a yellow coupler N-609, in the other light-sensitive layer 500 g of a dispersion of a cyan coupler ZG-97 and in the third light-sensitive layer 550 g of a dispersion of magenta couplers ZP-24 and N-651. The properties are represented in the table.

### Example 21.

False colour silver halide photographic material is prepared similarly to example 16, but in the one light-sensitive layer as sensitizing dye the compound (III) (A = C₂H₅, B = 4,5-benzo, B¹ = 5-OCH₃, R = R¹-(CH₂)₃SO₃, [K]⁺ = 3,3'-diethylthiazolyneocarbocyanine) in amount of 130 ml of 0,1 % alcohol solution is added and in the other layer the compound (I) (A = A²-H, A¹ = O-i-C₃H₇, R = R¹ = C₂H₅, n = 1, X = J) in an amount of 35 ml of 0,02% alcohol solution is added.

### Example 22.

False colour silver halide photographic material is prepared similarly to example 19, but before introduction of a dispersion of a yellow coupler in the one light-sensitive layer as a sensitizing dye a compound (III) (A = C₂H₅, B = 4,5-benzo, B¹ = 5-Cl, R = R¹ = (CH₂)₃SO₃), [K⁺] - N⁺H (C₂H₅)₃) in an amount of 140 ml of 0,1% alcohol solution is added and in the other layer as a sensitizing dye a compound (I) (A² = CH₃, A and A¹ together - CH₂C(CH₃)₂CH₂, R = R' = C₂H₅, B = 5,5'-di-OCH₃, 6,6'-di-SCH₃, X = CH₃SO₃⁻) is added.

### Example 23.

It is similar to an example 22, but in the one light-sensitive layer as a sensitizing dye it is added the compound (I) (A and A¹ = CHC(CH₃)₂CH₂, A² = H, R = R¹ = (CH₂)₃SO₃⁻, X = Na) in an amount of 100 ml of 0,02 % alcohol solution, and in the other layer it is added the compound of the formula (III) (A = C₂H₅, B = 4,5 = benzo, B¹ = 5-CH₃, R = (CH₂)₃SO₃⁻, R' = CH₂CH(OH)CH₂SO₃, [K]⁺ = HN⁺(C₂H₅)₃) in an amount of 50 ml of 0,05 % alcohol solution.

As it follows from the table, the false colour material according to the invention has a high resolving power (R = 140-145 MM⁻¹), i.e. higher than material according to the prototype (R = 68 MM⁻¹) and higher light sensitivity. This effect is achieved by application in a material of special silver halide emulsions or their mixtures, spectral sensitizers and/or their compositions, ensuring a variation of sensitization zone as well as application of appropriate activators of spectral sensitization and stabilizers.

This invention can be applied in a photographic industry for production of colour photographic materials used for registration of objects in visible and infra-red area of a spectrum.

**Table**

| Example | Sensitometric properties | | | Resolving power, R, mm⁻¹ |
|---|---|---|---|---|
| | Sensitivity, S_{0.85} | Contrast coefficient, γ | Fog density, Dₒ | |
| 1 | 30 | 1.6 | 0.30 | 68 |
| 2 | 130 | 2.4 | 0.25 | 110 |
| 3 | 200 | 2.0 | 0.20 | 100 |
| 4 | 200 | 2.2 | 0.20 | 110 |
| 5 | 250 | 2.0 | 0.20 | 145 |
| 6 | 270 | 2.2 | 0.15 | 145 |
| 7 | 310 | 2.8 | 0.25 | 120 |
| 8 | 250 | 2.0 | 0.15 | 145 |
| 9 | 300 | 2.3 | 0.18 | 145 |
| 10 | 400 | 2.2 | 0.25 | 100 |
| 11 | 320 | 1.9 | 0.17 | 120 |
| 12 | 500 | 2.1 | 0.21 | 110 |
| 13 | 480 | 2.0 | 0.16 | 110 |
| 14 | 700 | 1.7 | 0.25 | 100 |
| 15 | 600 | 2.3 | 0.20 | 110 |
| 16 | 600 | 1.8 | 0.21 | 110 |
| 17 | 600 | 1.95 | 0.20 | 110 |
| 18 | 600 | 1.95 | 0.20 | 110 |
| 19 | 200 | 1.9 | 0.20 | 120 |
| 20 | 250 | 1.9 | 0.23 | 110 |
| 21 | 550 | 1.9 | 0.20 | 110 |
| 22 | 250 | 1.9 | 0.20 | 120 |
| 23 | 300 | 2.0 | 0.18 | 135 |

## Claims

1. False colour silver halide photographic material consisting of a polymeric support on which on the one side antihalo backing layer is coated, on the other side at least two light-sensitive layers prepared from the silver halide photographic emulsion, containing colour forming couplers and infra-red, orthochromatic and/or panchromatic sensitizing dyes, auxiliary and protective gelatin layers are coated distinctive by that all light-sensitive layers are prepared from silver bromide-iodide emulsion with octahedral or flattened microcrystals with an average grain size 0,5-1,5 µm or their mixture and one of the light-sensitive layers contains as an infrared sensitizing dye one or more one compounds of the formula (1) where A = H; A¹ = OCH₂CH₂CH₂SO₃ ⁻; R = lower alkyl; A and A¹ together = CH₂C(CH₃)₂CH₂⁻; A² = H, lower alkyl; B = H, 5,5'-di-OCH₃, 6,6'-di-SCH₃ ; R = lower alcyl, (CH₂)₃SO₃⁻; n = 0,1; X = CH₃C₆H₄ SO₃ ⁻,J⁻, CH₃SO₃⁻, alkaline metal or is absent;
the second light-sensitive layer contains as an orthochromatic sensitizing dye more than one compounds of the formula (II): where Y = 0, N; A = lower alkyl or is absent; A¹ = H, lower alkyl, B = 5,5'--COOC₂H₅, 5,5 '-C₆H₅; R, R¹ = lower alkyl, (CH₂)₃SO₃⁻; [K]⁺ = NHC₅H₅ or is absent,
and/or the third light-sensitive layer contains as panchromatic sensitizing dye one or more compounds of the formula (III): where A = lower alkyl; B = 4,5-benzo, 4,5-tieno; B¹ = 5-OCH₃, 5-C₆H₅, 4'5'-benzo,5-Cl, 5-CH₃ ; R, R¹ = lower alkyl, (CH₂)₃SO₃⁻ ; [K]⁺ = HN⁺(C₂H₅)₃, HN⁺(C₄H₉)₃, C₅H₅-N⁺H, the alkaline metal, 3,3'-diethylthiazolinocarbocyanine, or is absent, and between light-sensitive layers auxiliary gelatin layers containing hardener are coated.

2. False colour silver halide photographic material on p.1 distinctive by that the light-sensitive layers contain as activators of spectral sensitization diperchporate of 3,3'-[1",2"-bis(ethoxy)-ethyl]-bis-(1-ethylbenzoimidazolium), or disodium salt of 4,4'-bis(4",6- phenoxy-1,3,5-triazinyl-2-amino)stilbene-2,2'-disulfonic acid or monosodium salt of 2-mercaptobenzoxazole-5-sulfonic acid.

3. False colour silver halide photographic material on p. 1 distinctive by that auxiliary gelatin layers contain as a hardener derivatives of triazine-1,3,5.

4. False colour silver halide photographic material on p. 1 distinctive by that the light-sensitive layers contain a mixture of silver bromide-iodide photographic emulsion with octahedral microcrystals and silver bromide-iodide photographic emulsion with flattened microcrystals in the ratio 1:9-9:1.
